

Dec. 5, 1961

T. L. HARRINGTON ET AL

3,011,412

SAFETY MARKING SYSTEM

Filed April 11, 1957

FIG. 1



FIG. 2



FIG. 3



INVENTORS

THOMAS L. HARRINGTON  
DONALD E. PEDERSON

BY

Carpenter, Abbott, Coulter & Kinney  
ATTORNEYS

# United States Patent Office

3,011,412

Patented Dec. 5, 1961

1

3,011,412

## SAFETY MARKING SYSTEM

Thomas L. Harrington, St. Paul, and Donald E. Pederson, White Bear Lake, Minn., assignors to Minnesota Mining and Manufacturing Company, St. Paul, Minn., a corporation of Delaware

Filed Apr. 11, 1957, Ser. No. 652,290

7 Claims. (Cl. 94—1.5)

This invention relates to an instant dry lane marking system, and more particularly relates to a method for marking traffic-ways such as aircraft runways, streets, highways and the like with durable, wear-resistant, guidelines, cross-walk, center-line and other safety indicia or stripes in a rapid manner so as not to interfere more than momentarily with the flow of traffic on the traffic-way. Our invention also relates to structures formed by the practice of our method.

The marking of aircraft runways, streets, highways, and the like, herein called "traffic-ways," with appropriate visual safety indicia has increasingly become a serious problem in recent years because of the necessity for avoiding lengthy interruptions to the flow of traffic. Instead of lessening, indications are that this problem will become more and more serious as traffic increases.

It is now well recognized, from the safety standpoint, that old marking methods which require rather lengthy interruption and re-routing of traffic during the time of application, and for so long a period thereafter as may be required for drying, frequently create as many safety problems as the resulting markings help to solve. Recently, some reduction of the time required for marking has been gained by the use of quick-drying materials, but such materials frequently do not retain desired appearance properties and rarely possess the requisite durability and wear-resistance so as to provide reasonably long lasting markings.

Another attack on this marking problems has involved the use of prefabricated cross-strips for application to traffic-ways. While this expedient to some extent reduces the time of traffic interruption required for marking, it is expensive and beyond the reach of many municipalities. Also, these prefabricated strips sometimes break loose from an underlying street surface, or are torn or removed by vandals.

According to our invention, painted safety markings of a vandal-proof, highly durable and wear-resistant quality may be provided on traffic-ways without more than momentarily interrupting the flow of traffic thereover. In fact, where safety markings, e.g., cross-lane strips, are to be applied at an intersection controlled by semaphore signals, interference with the flow of traffic can be said to be substantially eliminated, inasmuch as the requisite markings can be applied and made traffic-sustaining during the time required for one or two changes of signal.

By practicing our invention, street markings are formed which have a characteristic new and novel structure, being in part durable, wear-resistant and vandal-proof, and in part temporary or passing. Almost immediately after being formed, our structures can withstand traffic abrasion and the like without being disrupted or destroyed. After a relatively short but variable period of time, the structure is altered, not undesirably, and loses that part which is temporary or passing.

While the problem of providing durable safety markings in an economical manner and so as not to interfere more than momentarily with the flow of traffic has existed for many years, and while the preferred material for use in forming the temporary part of our structures has been known for years, no one to our knowledge has ever heretofore successfully presented the art with such

2

a rapid and efficient method of safety marking as herein set forth.

Our invention also introduces considerable economy in the art of providing superior safety markings for traffic-ways; and in this respect, it will be of great benefit to the taxpaying public.

The vandal-proof, durable and wear-resistant portion of our safety marking structures is that part which constitutes what we term the permanent safety marking. It is formed using self-hardening, resin-base paints, and may contain coloring pigments, as well as other ingredients, e.g., autocollimating units, where special properties as imparted by the ingredients are desired.

The temporary or passing portion of our marking structures is formed from material which is at least semi-transparent, and which almost immediately upon application becomes sufficiently tough and wear-resistant so as to withstand traffic abrasion and the like for at least a few hours without being destroyed or otherwise failing, yet is readily removed, as by water washing, without creating any traffic hazard or nuisance.

In the drawings made a part hereof, the structure of street markings of our invention is graphically illustrated.

FIGURE 1 is a plan view of a street marked with a center line.

FIGURE 2 is an enlarged cross section through line 2—2 of FIGURE 1.

FIGURE 3 is an enlarged cross sectional view of a safety marking structure, formed according to our invention, containing autocollimating elements.

Referring to FIGURES 1 and 2, the structures illustrated comprise a street surface 10, a permanent safety marking or paint layer 11, and a protective layer 12. In FIGURE 3 the same respective components are correspondingly numbered for the structure illustrated. Additionally, autocollimating elements 13, e.g., small glass reflex light-reflecting spheres or beads (see Heltzer Patent 2,574,971) are shown embedded within the pigmented, permanent marking layer 11. As described in the aforementioned Heltzer patent, these autocollimating elements will become operative to direct light back in a cone toward its source after paint on the top surface thereof is worn away by traffic abrasion. As an alternative, these autocollimating elements may be pressed into layer 11 (see Shuger Patent 2,268,537). Other components, of course, may be included in the permanent safety markings formed according to our invention, the structure in FIGURE 3 being merely illustrative.

In forming safety markings rapidly and in the manner contemplated by this invention, a self-hardening resin-base paint is applied in liquid condition to a previously cleaned road surface in a line or other marking, as desired, and thereafter while the paint is still in an unset or unhardened condition, i.e., before it has hardened to the point where it is non-tacky and can withstand traffic without becoming smeared and dirty, a coating of urea is applied thereover as a layer. The urea is applied from a hot, fluid melt and quickly cools and solidifies to form a protective skin over the applied paint strip, protecting the paint during the time it requires for hardening to a non-tacky, durable state. Within seconds after the urea has been applied as a protective layer, traffic may pass over the safety marking structure without causing the paint marking to become dirty or smeared.

The resin-base paint which forms the durable, wear-resistant, "permanent" safety markings of our structures must be of the type which does not require exposure to air to harden or set to a non-tacky, solid, durable condition. Thus, conventional drying oil base paints containing volatile solvents are unsuitable as a class to employ in the practice of this invention. When coated over

with urea, these drying oil paints containing solvents are sealed from the air and remain unset or unhardened for so long a time as the seal is maintained. For the practice of this invention, preferred paints to employ are those which are self-curing, i.e., autogenously curable, into hard but flexible, tough, non-tacky films, without the necessity for exposure to air, or the necessity for evaporation of solvent from their mixture. Suitable paints to employ in the practice of our method, although less desired than the



self-curing resin-base paints, are those formed from thermoplastic resins. Such thermoplastic resin-base paints contain little or no volatile solvent. After being applied in the molten state, they slowly cool, and thereby harden to a non-tacky, durable state after a period of time, usually at least about one-half hour.

As the temporary top coat we have found that the substance urea possesses a surprisingly excellent group of properties for use. It melts at about 132° C., well above the maximum ambient temperature where street markings are applied, and is easily held in fluid condition by raising it to about 150° C. for practical operations as herein discussed. Preferably it is not raised above about 160° C., at which temperature substantial decomposition of the urea is in evidence and odors may become objectionable. Experience has shown that, under varied temperature conditions, urea does not enter into reaction with a wide variety of suitable resin-base paints for use in the practice of our invention. It is easily applied as a hot fluid melt over flowable, unset resin-base paint markings, does not smear the paint markings, and rapidly cools to form a hard, tough, traffic-sustaining layer over the markings. The hardened crystalline urea layer stands up for a sufficient time under the flow of traffic so as to protect the resin-base paint markings from contact with traffic during the time needed for their hardening to a tough, abrasion-resistant and wear-resistant solid state. Further, the cooled and solid urea layer is semi-transparent and colorless so that the color of the marking is not obscured during the time it is weak and needs protection.

Of practical importance is the fact that urea layers are readily removed from a marking after their protective function is no longer needed, i.e., after the paint markings have hardened to a non-tacky, traffic-resistant state. The removal of the urea layer creates no problem. Rain falling on it will dissolve the urea and wash it away. If desired, one may remove it by street washing. The paint markings remain as clean and brightly colored indicia.

As an additional advantageous property of applied urea layers may be cited the fact that they are odorless and are not offensive to the public. During the time of the layer's protective function as well as during its removal by water washing, no traffic hazard such as slipperiness is created.

The following examples are offered to illustrate the teachings herein, but are not to be construed as limitative of this invention. Unless otherwise noted, all parts are by weight.

#### EXAMPLE 1

| Mixture A                      | Parts |
|--------------------------------|-------|
| Epoxy resin ("Epon 828")       | 189   |
| Pigment grade titanium dioxide | 81    |
| Methyl amyl acrylate monomers  | 20.5  |

#### Mixture B

|                                 |     |
|---------------------------------|-----|
| Polyamid resin ("Versamid 125") | 197 |
| Methyl amyl acrylate monomers   | 63  |

The epoxy resin was obtained commercially from the Shell Development Company under the trade name "Epon

828." This resin is a liquid epoxy resin having an average of more than one 1,2 epoxy group in the molecule. Typical epoxy resins of this type may be produced by the reaction of 2,2-bis(4-hydroxyphenyl) propane (i.e., Bisphenol A) and epichlorohydrin in alkaline media at elevated temperatures within the approximate range of about 50-150° C. While the resins are complex mixtures rather than a single chemical compound, they may be represented by the illustrative formula



15 where *n* has an average value between zero and about 7, depending for the most part on the relative proportions of Bisphenol A and epichlorohydrin in the initial reaction mixture, the larger amounts of epichlorohydrin being used to prepare liquid epoxy resins. Other polyhydric phenols, e.g. resorcinol, 2,2-bis(4-hydroxyphenyl)-butane, and various tris-phenols, may be substituted for the Bisphenol A. Various other polyhydroxy compounds may likewise be substituted, by appropriate known procedures, for the polyhydric phenols in preparing analogous resinous base materials, ethylene glycol and glycerine being typical examples. "Epon 828" is but one illustrative suitable liquid epoxy resin (melting at about 8 to 12° C.). It has a Gardner-Holt viscosity at 25° C. of Z5 to Z6, and an epoxide equivalence of about 190 to 210. In other words, about 190 to 210 grams of this resin contain 1 gram equivalent of epoxide.

20 The polyamid resin of the above formula reacts with the epoxy resin to promote hardening of the composition, and is the addition product of polymerized long chain fatty acids and polyfunctional primary and secondary amines. "Versamid 125" is stated by the manufacturer, General Mills, Inc., to have an average molecular weight of about 2,000, an acid number of 7, and a Brookfield viscosity of about 45,000 to 55,000 centipoises at 23° C.

25 Methyl amyl acrylate monomers may be prepared by ester reaction between acrylic acid and methyl amyl alcohol (methyl isobutyl carbinol).

30 About 100 parts of Mixture A and 43.3 parts of Mixture B, together with 14 parts additional of methyl amyl acrylate monomers, and 5 parts of diethylene triamine 35 curing agent for the epoxy resin, were blended together by stirring, and then sprayed onto a concrete road surface through a conventional spraying machine nozzle in stripes or lines having a thickness of about 0.027 inch and a width of about 6 inches. About one gallon of the mix was used to form lines and stripes having a total surface area of 60 square feet. Immediately after application, molten urea held at about 150° C. was poured over the applied paint film, using about 4 or 5 gallons 40 of molten urea (i.e., about 50 pounds) to cover the stripes or lines formed using one gallon of paint. The large quantity of urea employed served to cover all areas of the painted stripes as a layer even though molten urea shows some tendency, when attempts are 45 made to apply it as an extremely thin layer, to crawl off the painted stripes. Within about 30 seconds after the molten urea was applied, it had hardened sufficiently to 50 provide a protective layer completely covering the painted markings. Vehicles were driven over the markings, without damage to the same, the urea layer serving to protect 55 the markings from traffic contact.

60 After about 8 hours of protection, the painted markings of this example had cured sufficiently so that the urea could be removed leaving a permanent durable and non-smudged safety marking. Removal of the urea was 65 accomplished by rain, which fell about 8 hours after application. The rain water dissolved the urea and washed it away. No traffic hazard or public nuisance was created.

70 Using the compositions of this example, the foregoing

method was employed to mark asphalt and cobblestone street surfaces, and gave the desired results as afore-indicated.

The paint composition illustrated in this example has a relatively short pot life during which it remains at a suitable consistency for spray application, as afore-described, the pot life being only about one hour after all ingredients are mixed together; therefore, in using this paint composition in practice, the amount of paint mixed for application should not exceed the amount easily applied within the first hour after the formula is prepared.

## EXAMPLE 2

|                                                                                                | Parts |
|------------------------------------------------------------------------------------------------|-------|
| Epoxy resin ("Epon 1004")                                                                      | 15.6  |
| Dibutyl phthalate plasticizer                                                                  | 6.7   |
| Pigment grade calcium carbonate ("Atomite")                                                    | 18    |
| Pigment grade titanium dioxide ("Unitan OR150")                                                | 12    |
| Small glass beads having a diameter of about 2.5 to 7 mils and a refractive index of about 1.5 | 47.7  |

The epoxy resin of this example, while formed using materials such as set forth in Example 1, was formed with less epichlorhydrin in the reaction mixture so as to produce a resin which remains as a solid at room temperature. "Epon 1004" melts at about 95-105° C., and has an epoxide equivalency from about 870 to 1025.

All the ingredients above, including the beads, were mixed together by kneading action at a temperature of 175° F. until a uniform smooth blend containing the glass beads was formed. The blend was poured into pails and allowed to cool.

To about 17 parts of the above batch was added about one part of phthalic anhydride, which serves as a curing or hardening accelerator for the composition. This mixture was then melted by heating to about 220° F., and the phthalic anhydride blended therein. While hot, the mixture was knife coated on a concrete roadway in the form of safety marking lines. One gallon of the mix was used to form stripes totalling about 40 square feet in surface area. The applied paint cooled rapidly and solidified on cooling to a tacky, semi-solid state. Hot molten urea was flute sprayed immediately over the markings in a sufficient amount to form a thin urea layer covering the total area of the markings except for a short strip which was left free of urea. About one minute after the urea was applied, traffic was allowed to pass over all areas of the marking strips, both those covered with urea and those left uncovered. Traffic over the strip free of urea caused it to be smeared and to pick up dirt, whereas the urea protected markings were left free of smearing and dirt. After about one hour the urea layer could be removed by water washing without the underlying paint film becoming smeared or dirty as a result of subsequent traffic contact.

While the paint of this example, even with added anhydride, requires several weeks to cure at room temperature, its surface stickiness is substantially killed by the hot melt application of urea thereover, which serves to heat the exposed and urea contacted surface areas of the paint film and accelerate curing of such surface areas, thus providing a thin essentially non-tacky skin of cured paint over the underlying portion of paint which takes longer to cure. Shortly after the urea has been applied to this paint film, therefore, its protective function is no longer needed and it may be removed.

## EXAMPLE 3

The composition and procedure of Example 1 were employed except that 14 parts of methyl ethyl ketone solvent were substituted for the 14 parts of additional methyl amyl acrylate monomers in the paint formula. The methyl ethyl ketone in this formulation does not enter into reaction with the other components of the paint formula (as happens in the formula of Example 1), and is entrapped in the finally cured paint markings as a volatile solvent. Despite this fact, the marking

strips and lines formed from this paint composition, while weaker and softer than those of Example 1, were firm enough to withstand traffic and were about equal to the markings of Example 1 with respect to their ability to resist damage by traffic.

As in the procedure employed in Example 1, the paint of this example was applied in stripes on a road surface—in this case an asphalt surface—and coated over with a layer of urea. Subsequently the urea was washed away after the underlying paint film was cured.

## EXAMPLE 4

The composition and procedure of Example 1 were used except that styrene oxide monomers were substituted on a weight for weight basis for all of the methyl amyl acrylate monomers of Example 1. Styrene oxide, like methyl amyl acrylate, serves as a reactive diluent in this composition, entering into reaction (an addition reaction as distinguished from a condensation reaction) with other components of the paint mix during hardening, and becoming an integral part of the resulting marking. In all respects this composition performed as illustrated for the markings of Example 1. Hot melted urea was used as a top coat, as described in Example 1.

## EXAMPLE 5

The following paint formulation illustrates the use of a method of this invention with self-hardening resin-base paints which may be characterized as thermoplastic paint mixtures:

|                                                     | Parts |
|-----------------------------------------------------|-------|
| Rosin                                               | 58.4  |
| Alkyd resin                                         | 10.7  |
| Dioctyl phthalate plasticizer                       | 3     |
| Titanium dioxide pigment ("Titanox RCHT")           | 30    |
| Pigment grade calcium carbonate filler              | 30    |
| Glass beads of the character described in Example 2 | 168   |

The alkyd resin was an oil-modified glycerol phthalate prepared from a mixture of at least 31% phthalic anhydride by weight and about 57% soya oil with the remainder being essentially glycerol. This resin has a Gardner-Holt viscosity of I to L, and an acid number between 6 and 14.

The titanium dioxide pigment here employed was a calcium modified pigment formed by precipitating titanium dioxide onto finely divided calcium sulfate, and consists of about 70% calcium sulfate as the core of pigment particles, with about 30% titanium dioxide occupying surface areas of the particles. This pigment is merely illustrative of one type to employ. Many others are suitable.

The paint formulation of the example was maintained in a hot fluid condition by heating it to a 275° F. for application to roadways. It was knife coated in stripes on a concrete roadway; and immediately after application, hot molten urea was poured upon it. The urea cooled to form a protective layer within about one minute after application, and traffic was allowed to pass over the marking. No damage to the marking occurred. After about one hour, which is a sufficiently lengthy period of time for this paint film to lose its tack and harden into a solid durable film, the urea could be removed, e.g., by spraying water over the structure, and the markings were found to be highly traffic-resistant.

It will be readily appreciated by those skilled in the art that many varied self-hardening resin-base paints may be used in the practice of this invention, and that these may be modified extensively by additions of various materials and ingredients to achieve special effects in the resulting marking. Resins such as isocyanates, polyamids, and various polyesters, are illustrative ones which may be employed as the base for paint formulations useful in the practice of this invention. Curing agents of a wide variety, as well understood in the self-curing resin art,

may be useful. Pigments may vary. While white has become a popular marking pigment, as illustrated in the examples, yellow lead chromate is frequently employed. Many others, however, will be found to function equally as well in the practice of the invention.

The foregoing is intended to illustrate but not limit our invention, and all equivalents are fully comprehended.

That which is claimed is:

1. The method of providing clean, sharply outlined, traffic-resistant markings on traffic-way surfaces with no more than momentary interruption of traffic over said surfaces, comprising applying to a desired area of the surface a thin coating of a self-hardening spreadable liquid resin-base paint marking composition, applying thereover as a melt a continuous layer of hard, brittle, water-soluble crystalline urea material melting at a temperature well above the maximum ambient temperature and below the temperature at which degradation of the marking composition is obtained, said crystalline material being applied in a continuous layer over said marking composition before said marking composition has hardened sufficiently to sustain traffic and permitting the melt to solidify.

2. The method of claim 1 in which the marking composition is rapidly heat-curing and at least the surface of the thin coating is accelerated in curing during contact with the applied molten crystalline material.

3. The method of claim 1 in which the marking composition is thermoplastic and hardens and slowly loses surface tackiness on cooling from plastic condition.

4. A method for providing durable, wear-resistant, clean, visual, safety markings on traffic-ways in such manner as not to interfere more than momentarily with the flow of traffic thereover, said method including the step of applying a layer of urea over a self-hardening resin-base paint marking substantially immediately after said marking has been applied from fluid composition to said traffic-way, said urea being applied over said marking as a hot, melted fluid which cools rapidly upon application to form a temporary, traffic-sustaining, easily-removed, non-hazardous, water-soluble, protective layer

over said marking, thereby to protect said marking from dirt and traffic contact during the time required by said marking to set to a durable, traffic-resistant state.

5. A method of applying durable, wear-resistant, clean, visual, safety markings on traffic-ways in such manner as not to interfere more than momentarily with the flow of traffic thereover, said method comprising applying upon the surface of a traffic-way a safety marking of a pigmented, self-hardening, resin-base paint, and applying urea as a layer over said marking substantially immediately after forming said marking, said urea being applied over said marking from a hot, fluid melt which cools rapidly upon application to form a temporary, traffic-sustaining, easily-removed, non-hazardous, water-soluble, protective layer over said marking, thereby to protect said marking from traffic contact during the time required by said marking to harden to a durable, traffic-resistant state.

6. On a traffic-way: traffic markings of self-hardening resin-base paint composition temporarily protected by a hardened continuous transparent protective surface layer of urea, said urea being non-reactive with said self-hardening composition.

7. A structure comprising a hard surfaced traffic-way, a layer of pigmented, non-tacky, self-hardenable, tough, flexible and durable, resin-base paint on said traffic-way, and a temporary protective, traffic-sustaining layer of cool and hardened urea over said paint on said traffic-way, said urea layer being non-reactive with said paint on said traffic-way and being easily dissolved by water and washed away from said structure without creating traffic hazards and offensive odors.

References Cited in the file of this patent

UNITED STATES PATENTS

|           |          |               |
|-----------|----------|---------------|
| 2,408,814 | Selden   | Oct. 8, 1946  |
| 2,420,720 | Pechukas | May 20, 1947  |
| 2,574,971 | Heltzer  | Nov. 13, 1951 |
| 2,680,595 | Upham    | June 8, 1954  |
| 2,898,825 | Walker   | Aug. 11, 1959 |